

# United States Patent Office

2,842,462

Patented July 8, 1958

1

2,842,462

## ANTISTATIC SYNTHETIC TEXTILE MATERIAL

Hermann Haas, Hans Markert, and Gustav Lietz, Dusseldorf, Germany, assignors to Böhme Fettchemie G. m. b. H., Dusseldorf, Germany, a corporation of Germany

No Drawing. Application December 16, 1954  
Serial No. 475,812

Claims priority, application Germany December 21, 1953

4 Claims. (Cl. 117—139.5)

This invention relates to antistatic preparations and to a process of treating textile materials, and more particularly synthetic textile materials or mixtures of synthetic and natural fibers, with such preparations so as to prevent generation and accumulation of static electricity in said textile materials.

It is known that textile materials composed of synthetic fibers often accumulate disturbing electric charges on working and processing or using such materials. This property of generating and accumulating static electricity is especially pronounced in materials made from polycondensation products, such as polyesters, polyamides, and the like; from vinyl polymerization products, such as polyvinyl chloride, polyvinyl acetate, and the like; from polymers of acrylic acid derivatives, such as polymers of acrylic acid esters, acrylonitrile, and the like. Natural fibers containing nitrogen, such as silk and wool, are also subject to the generation and accumulation of static electrical charges at least to a certain extent.

Generation of static electricity and accumulation of electric charges considerably interfere with mechanical processing of said materials and are an inconvenience in their use. For example, in carding, drawing and spinning of such fibers, static electricity can be generated to such an extent that further processing will be rendered impossible because, due to such accumulation of electric charges, the individual fibers are caused to spread, loose fibers may be attracted to or repelled from the fibers being worked and the spinning material may become wrapped upon rotating parts of the processing machines. Woven and knitted fabrics made from such fibers can often be processed and packed only with great difficulty. On wearing finished garments of such materials, such garments either adhere and cling to each other and to the wearer or they repel each other in an undesired and objectionable manner.

It is one object of the present invention to provide a simple and effective process of preventing generation and accumulation of static electricity in textile materials, or of eliminating or at least considerably reducing static charges generated or accumulated therein.

Another object of the present invention is to provide preparations for the treatment of synthetic fiber materials, which preparations prevent generation and accumulation of static electricity in said fibers on subsequent spinning and further processing.

A further object of the present invention is to provide an impregnating preparation for the treatment of finished woven or knitted fabrics made of synthetic fiber material, said impregnating preparation safeguarding such fabrics against accumulation of static charges.

Still another object of the present invention is to provide synthetic fiber material which is substantially free of static electricity and does not develop static charges on processing it and on wearing garments or using products made therefrom.

Various other objects and advantages of our invention will become apparent as this description proceeds.

2

In principle, the present invention consists in treating the textile material during its manufacture, during processing and finishing, or during its use with neutral alkylene oxide addition compounds of acid phosphoric acid esters of higher molecular hydroxyl compounds. As a result of such a treatment, generation and accumulation of static electricity in said textile materials are prevented or at least reduced to such an extent that it has no more disturbing effect on processing and using said materials.

10 The antistatic preparations used for the treatment of textile materials and more particularly of synthetic textile materials are preferably aqueous solutions or dispersions of such alkylene oxide addition compounds of acid phosphoric acid esters of higher molecular hydroxyl compounds. Such aqueous solutions or dispersions must contain at least about 1 g. of said addition compounds per liter. Amounts between about 1 g. and about 50 g. per liter are ordinarily sufficient to produce the desired effect. Higher concentrations may, of course, also be employed but usually will serve no useful purpose.

15 It is understood that the concentration of the addition compound in the aqueous solution or dispersion depends upon the type of textile material to be treated and the method of treatment to be employed. It is readily possible to determine by simple preliminary tests the optimum concentration of the addition compound which should be used for each preparation, for each textile material and for each method of treatment.

20 One of the methods advantageously used in this treatment comprises spraying or sprinkling the fiber material, for instance, in the form of staple fiber on conveyer belts, with antistatic solutions or dispersions according to the present invention, or the textile material may be sprayed therewith in suitable chambers from which unabsorbed treatment material may be recovered, or it may be dipped or immersed into said solutions or dispersions.

25 The antistatic treatment can also be effected during winding, spooling, doubling, twisting, and the like operations, by using spooling and spinning oils containing such antistatic addition compounds.

30 Where necessary, known emulsifier and dispersing agents may be added to the antistatic preparations according to the present invention; also hygroscopic agents, lubricants, brightening agents and other agents facilitating further processing and imparting to the treated textile materials additional improving effects may be used. Mineral, animal or vegetable oils, fats or waxes which are held in emulsion by said antistatic alkylene oxide addition compounds may be used as lubricants in the textile processing operations. As hygroscopic agents there may be employed, for instance, glycerol, glycols, urea or hygroscopic inorganic salts, together with the alkylene oxide antistatic agents described herein.

35 The acid phosphoric acid esters used in the production of the alkylene oxide addition compounds forming the basis of the new antistatic preparations described herein may be produced according to methods known per se, for instance, by esterifying higher molecular alcohols with phosphorus pentoxide, pyrophosphoric acid, metaphosphoric acid and other phosphoric acids containing less water in their molecule than pyrophosphoric acid, as well as with mixtures of such acids or with phosphorus oxychloride.

40 Said acid esters are converted into their alkylene oxide addition compounds, i. e. the corresponding neutral mixed esters, by the addition of alkylene oxides, especially of ethylene oxide, at a temperature between about 50° C. and about 100° C. in the absence of catalysts. Thereby 1 to 4 or even more mols of ethylene oxide are added to each available acid group of the ester used as one of the reaction components.

45 As starting materials for the preparation of the acid

phosphoric acid esters there are employed aliphatic, cycloaliphatic, cycloaliphatic-aromatic, and aliphatic-aromatic hydroxyl compounds with at least 6 carbon atoms in their molecule, such as hexanol, octanol, dodecanol, oleyl alcohol, octadecanol, cyclohexanol, alkyl cyclohexyl alcohols, naphthene alcohols, benzyl alcohol, tetrahydro-naphthol, decahydronaphthol, alkyl phenols and the like hydroxyl compounds. The hydroxyl compounds may also contain substituents or their hydrocarbon chain may be interrupted by hetero atoms, such as oxygen, sulfur, or nitrogen, or by hetero atom groups derived from said hetero atoms.

As alkylene oxide there is primarily used ethylene oxide, but propylene oxide, glycidyl, and the like alkylene compounds may also be employed.

Alkylene oxide addition compounds of acid phosphoric acid esters as they are contained in antistatic preparations produced according to the present invention may be, for instance, the following compounds:

The condensation product of 2 mols of a technical grade mixture of hexadecanol and octadecanol with 1 mol of phosphorus pentoxide and 5 to 7 mols of ethylene oxide; the condensation product of 2 mols of octadecanol with 1 mol of phosphorus pentoxide and 4 to 8 mols of ethylene oxide; the condensation product of 1.5 mols of dodecanol with 1 mol of phosphorus pentoxide and 6 to 10 mols of ethylene oxide; and similar compounds based upon the use of hydroxyl compounds such as specified above.

The following examples serve to illustrate the present invention without, however, limiting the same thereto.

#### Example I

Cut staple fibers of polyvinyl chloride, polyamides, polyacrylonitrile, or polyesters are treated with an aqueous dispersion containing 5 g. per liter of a condensation product of 2 mols of a mixture of fatty alcohols having 16 and 18 carbon atoms in their molecules, 1 mol of phosphorus pentoxide, and 4 to 6 mols of ethylene oxide by sprinkling the fibers on a conveyor belt with said aqueous dispersion. Thereafter the treated fibers are centrifuged and dried in a conventional manner.

The resulting fibers do not generate and accumulate static electricity and can be processed with great ease by spinning.

#### Example II

Synthetic fibers as employed in Example I are treated, in the form of endless filaments, during winding, spooling, doubling, and twisting with spooling or spinning oils which contain, finely and uniformly dispersed therethrough, 3% of the condensation product of 2 mols of a fatty alcohol mixture  $C_{12}$ - $C_{18}$ , 1 mol of phosphorus pentoxide, and 4 to 8 mols of ethylene oxide. In this manner, antistatic finished yarns of excellent closeness of the twist and good elastic properties are obtained.

#### Example III

For spinning synthetic fibers as set forth in Example I in mixture with natural fibers such as wool or cotton, wool oils and spinning oils prepared, for instance, on the basis of fatty acids, fatty acid glycerides, and/or mineral oils, are conventionally used. According to the present invention 2% to 5% of the condensation product of 2 mols of decanol, 1 mol of phosphorus pentoxide, and 4 to 8 mols of ethylene oxide are added to such wool oils and spinning oils and are finely and uniformly dispersed therethrough. The resulting preparations not only impart satisfactory antistatic properties to yarns spun therewith but also excellent resistance against distortion and draft and warping, and yield yarns of uniform quality.

#### Example IV

Finished woven or knitted fabrics made of synthetic fibers of the classes heretofore set forth are impregnated with an aqueous dispersion of the condensation product of 2 mols of a mixture of fatty alcohols having 16 and 18 carbon atoms in their molecules, 1 mol of phosphorus pentoxide, and 4 to 6 mols of ethylene oxide, said dispersion containing 30 g. of said condensation product per liter. Impregnation is effected by treatment on a Foulard machine or similar sizing or impregnating device. The impregnated fabrics do not generate static electricity on friction and have an agreeable feel similar to that of natural fibers.

It is to be understood that many changes and variations in the composition of the antistatic preparations, in the components forming the neutral alkylene oxide addition compounds of acid phosphoric acid esters of higher molecular organic hydroxyl compounds, in the amounts of said addition compounds present in said preparations, in the methods of treating textile materials with said preparations, and in other features of our invention may be made without departing from the spirit of our invention or the scope of the following claims.

We claim:

1. An antistatic synthetic textile material impregnated with a neutral condensation product, formed by esterifying 1 mol phosphorus pentoxide with 2 mols of fatty alcohol with from 6 to 18 carbon atoms, and subjecting the resulting acid phosphoric acid ester to a condensation reaction with from 1 to 10 mols ethylene oxide at a temperature between 50 and 100° C., in an amount sufficient to impart antistatic properties to said synthetic textile material.

2. An antistatic synthetic textile material impregnated with a neutral condensation product, formed by esterifying 1 mol phosphorus pentoxide with 2 mols of a mixture of fatty alcohols having from 16 to 18 carbon atoms, and subjecting the resulting acid phosphoric acid ester to a condensation reaction with 4 to 6 mols ethylene oxide at a temperature between 50 and 100° C., in an amount sufficient to impart antistatic properties to said synthetic textile material.

3. An antistatic synthetic textile material impregnated with a neutral condensation product, formed by esterifying 1 mol phosphorus pentoxide with 2 mols of a mixture of fatty alcohols having from 12 to 18 carbon atoms, and subjecting the resulting acid phosphoric acid ester to a condensation reaction with 4 to 8 mols ethylene oxide at a temperature between 50 and 100° C., in a sufficient amount to impart antistatic properties to the textile material.

4. An antistatic synthetic textile material impregnated with a neutral condensation product, formed by esterifying 1 mol phosphorus pentoxide with 2 mols decanol, and subjecting the resulting acid phosphoric acid ester to a condensation reaction with 4 to 8 mols ethylene oxide at a temperature between 50 and 100° C., in an amount sufficient to impart antistatic properties to the textile material.

#### References Cited in the file of this patent

##### UNITED STATES PATENTS

- |           |                        |               |
|-----------|------------------------|---------------|
| 1,970,578 | Schoeller et al. ----- | Aug. 21, 1934 |
| 2,676,122 | McCarthy -----         | Apr. 20, 1954 |
| 2,729,576 | Trusler -----          | Jan. 3, 1956  |

##### FOREIGN PATENTS

- |         |               |               |
|---------|---------------|---------------|
| 498,262 | Belgium ----- | Oct. 14, 1950 |
|---------|---------------|---------------|